



US007527905B2

(12) **United States Patent**  
**Yu**

(10) **Patent No.:** **US 7,527,905 B2**  
(45) **Date of Patent:** **\*May 5, 2009**

(54) **IMAGING MEMBER**

(75) Inventor: **Robert C. U. Yu**, Webster, NY (US)

(73) Assignee: **Xerox Corporation**, Norwalk, CT (US)

(\*) Notice: Subject to any disclaimer, the term of this patent is extended or adjusted under 35 U.S.C. 154(b) by 393 days.

This patent is subject to a terminal disclaimer.

(21) Appl. No.: **11/425,179**

(22) Filed: **Jun. 20, 2006**

(65) **Prior Publication Data**

US 2007/0141488 A1 Jun. 21, 2007

**Related U.S. Application Data**

(63) Continuation-in-part of application No. 11/314,484, filed on Dec. 21, 2005.

(51) **Int. Cl.**

**G03G 15/04** (2006.01)

(52) **U.S. Cl.** ..... **430/64; 430/65; 430/60**

(58) **Field of Classification Search** ..... **430/64, 430/65, 60**

See application file for complete search history.

(56) **References Cited**

U.S. PATENT DOCUMENTS

- |             |         |                  |
|-------------|---------|------------------|
| 3,121,006 A | 2/1964  | Middleton et al. |
| 4,233,384 A | 11/1980 | Turner et al.    |
| 4,265,990 A | 5/1981  | Stolka et al.    |
| 4,286,033 A | 8/1981  | Neyhart et al.   |
| 4,291,110 A | 9/1981  | Lee              |
| 4,299,897 A | 11/1981 | Stolka et al.    |
| 4,306,008 A | 12/1981 | Pai et al.       |

|              |         |                   |
|--------------|---------|-------------------|
| 4,338,387 A  | 7/1982  | Hewitt            |
| 4,439,507 A  | 3/1984  | Pan et al.        |
| 4,587,189 A  | 5/1986  | Hor et al.        |
| 4,639,402 A  | 1/1987  | Mishra et al.     |
| 4,664,995 A  | 5/1987  | Horgan et al.     |
| 4,988,597 A  | 1/1991  | Spiewak et al.    |
| 5,055,366 A  | 10/1991 | Yu et al.         |
| 5,149,608 A  | 9/1992  | Deibler et al.    |
| 5,215,839 A  | 6/1993  | Yu                |
| 5,244,762 A  | 9/1993  | Spiewak et al.    |
| 5,378,566 A  | 1/1995  | Yu                |
| 5,571,649 A  | 11/1996 | Mishra et al.     |
| 5,576,130 A  | 11/1996 | Yu et al.         |
| 5,591,554 A  | 1/1997  | Mishra et al.     |
| 5,643,702 A  | 7/1997  | Yu                |
| 5,703,487 A  | 12/1997 | Mishra            |
| 5,830,614 A  | 11/1998 | Pai et al.        |
| 6,008,653 A  | 12/1999 | Popovic et al.    |
| 6,119,536 A  | 9/2000  | Popovic et al.    |
| 6,150,824 A  | 11/2000 | Mishra et al.     |
| 6,294,300 B1 | 9/2001  | Carmichael et al. |
| 6,326,111 B1 | 12/2001 | Chambers et al.   |
| 6,379,853 B1 | 4/2002  | Lin et al.        |

*Primary Examiner*—Mark A Chapman

(74) *Attorney, Agent, or Firm*—Eugene O. Palazzo; Fay Sharpe LLP

(57) **ABSTRACT**

An imaging member comprising a charge generating layer, a charge transport layers and an optional barrier layer between the charge generating layer and the charge transport layer. The charge transport layer may comprise a first and a second or more layers, wherein the first layer comprises a film-forming polymer having hole-transporting capability, but does not contain charge transport molecules. The barrier layer and/or the first charge transport layer reduces or prevents the buildup of charge transport molecules along the surface of the charge generating layer to thereby suppress the development of charge-deficient spots (CDS) defects in the imaging print-out copies from the imaging member.

**24 Claims, 4 Drawing Sheets**





FIG. 1



**FIG. 2**

**FIG. 3**

**FIG. 4**

**1**  
**IMAGING MEMBER**

This application is a continuation-in-part of U.S. patent application Ser. No. 11/314,484 filed on Dec. 21, 2005, incorporated herein by reference in its entirety.

BACKGROUND

There is disclosed herein, in various embodiments, an imaging member used in electrophotography that reduces or eliminates charge deficient spots. The imaging member includes a charge generating layer, an optional under-layer or barrier layer, and a charge transport layer. The concentration of charge transport molecules that are present in the under-layer and/or charge transport layer near the surface of the charge generating layer are reduced or eliminated. This minimizes or eliminates charge deficient spots.

A typical electrophotographic imaging member is imaged by uniformly depositing an electrostatic charge on an imaging surface of the electrophotographic imaging member and then exposing the imaging member to a pattern of activating electromagnetic radiation, such as light, which selectively dissipates the charge in the illuminated areas of the imaging member while leaving behind an electrostatic latent image in the non-illuminated areas. This electrostatic latent image may then be developed to form a visible image by depositing finely divided electroscopic marking toner particles on the imaging member surface. The resulting visible toner image can then be transferred to a suitable receiving member, such as paper.

A number of current electrophotographic imaging members are multilayered photoreceptors that, in a negative charging system, comprise a substrate support, an electrically conductive layer, an optional charge blocking layer, an optional adhesive layer, a charge generating layer, a charge transport layer, and optional protective or overcoating layer(s). Although multilayered photoreceptors can comprise several forms, for example, flexible belts, rigid drums, flexible scrolls, and the like, photoreceptors having a flexible belt configuration will be discussed and represented hereinafter for reason of simplicity. Flexible photoreceptor belts may either be seamed or seamless belts. An anti-curl layer may be employed on the back side of the flexible substrate support, the side opposite to the electrically active layers, to achieve desired photoreceptor belt flatness.

Although excellent toner images may be obtained with multilayered belt photoreceptors, a delicate balance in charging image and bias potentials, and characteristics of toner/developer must be maintained. This places additional constraints on photoreceptor manufacturing, and thus, on the manufacturing yield. Localized microdefect sites, varying in size of from about 5 to about 200 microns, can sometimes occur in manufacture and appear as print defects (microdefects) in the final imaged copy. In charged area development, where the charged areas are printed as dark areas, the sites print out as white spots. These microdefects are called microwhite spots. In discharged area development systems, where the exposed area (discharged area) is printed as dark areas, these sites print out as dark spots on a white background. All of these microdefects, which exhibit inordinately large dark decay, are called "charge deficient spots" (CDS). Since the microdefect sites are fixed in the photoreceptor, the spots are registered from one cycle of belt revolution to next. Charge deficient spots have been a serious problem for a very long time in many organic photoreceptors, such as multilayered photoreceptors where a pigment is dispersed in a matrix of a bisphenol Z type polycarbonate film forming binder.

**2**

Whether these localized microdefect or charge deficient spot sites will show up as print defects in the final document depends, to some degree, on the development system utilized and, thus, on the machine design selected. For example, some of the variables governing the final print quality include the surface potential of photoreceptor, the image potential of the photoreceptor, photoreceptor to development roller spacing, toner characteristics (such as size, charge, and the like), the bias applied to the development rollers and the like. The image potential depends on the light level selected for exposure. The defect sites are discharged, however, by the dark discharge rather than by the light. The copy quality from generation to generation is maintained in a machine by continuously adjusting some of the parameters with cycling. Thus, defect levels may also change with cycling.

Techniques have been developed for the detection of CDS's. These have largely involved destructive testing, although some contactless methods have been developed. Additionally, multilayer imaging members have been developed to block charge injection from the substrate which can give rise to CDS's.

The present disclosure is directed to producing an improved imaging member that reduces or eliminates charge deficient spots, among other characteristics.

CROSS REFERENCE TO RELATED  
APPLICATIONS

The following applications, the disclosures of each being totally incorporated herein by reference, are mentioned:

U.S. application Ser. No. 11/158,119, filed Jun. 21, 2005, entitled "Imaging Member," by Satchidanand Mishra, et al. discloses an imaging member having a charge transport layer in which the concentration of a charge transport component is at a peak in a region of the charge transport intermediate the first and second surfaces of the charge transport layer.

U.S. application Ser. No. 10/744,369, filed Dec. 23, 2003, entitled "Imaging Members," by Satchidanand Mishra, et al. discloses a charge transport layer in which the concentration of a charge transport component decreases, such as by a decreasing concentration gradient, from the lower surface to an upper surface in the charge transport layer.

U.S. application Ser. No. 10/736,864, filed Dec. 16, 2003, entitled "Imaging Members," by Anthony M. Horgan, et al. discloses a charge transport layer of an imaging member that includes a plurality of charge transport layers coated from solutions of similar or different compositions or concentrations, wherein the upper or additional transport layer or layers comprise a lower concentration of charge transport component than the first (bottom) charge transport layer.

U.S. application Ser. No. 10/320,808, filed Dec. 16, 2002, now U.S. Pat. No. 6,933,089 which issued on Aug. 23, 2005, entitled "Imaging Members," by Anthony M. Horgan et al discloses a dual charge transport layer in which the top layer comprises a hindered phenol dopant.

U.S. application Ser. No. 11/158,119, filed Jun. 21, 2005, entitled "Imaging Member," by Satchidanand Mishra, et al. discloses an imaging member having a charge transport layer in which the concentration of a charge transport component is at a peak in a region of the charge transport intermediate the first and second surfaces of the charge transport layer.

U.S. application Ser. No. 11/156,882, filed Jun. 20, 2005, entitled "Imaging Members" by Satchidanand Mishra, et al. discloses an imaging member incorporating an undercoat layer intermediate an imaging layer and an electrically conductive layer. The undercoat layer includes a film forming

polymer with a particulate material dispersed therein. The particulate material supports a charge blocking material thereon.

## INCORPORATION BY REFERENCE

The following patents, the disclosures of which are incorporated in their entireties by reference, are mentioned:

Electrophotographic imaging members having at least two electrically operative layers including a charge generating layer and a transport layer comprising a diamine are disclosed in U.S. Pat. Nos. 4,265,990; 4,233,384; 4,306,008; 4,299,897; and, 4,439,507.

U.S. Pat. No. 5,830,614 relates to a photoreceptor that comprises a support layer, a charge generating layer, and two charge transport layers. The first charge transport layer consists of charge transporting polymer comprising a polymer segment in direct linkage to a charge transporting segment and the second transport layer comprises a charge transporting polymer as in the first layer, but with a lower weight percentage of the charge transporting segment.

U.S. Pat. Nos. 5,591,554; 5,576,130; and, 5,571,649 disclose methods for preventing charge injection from substrates which give rise to CDS's. These patents disclose an electrophotographic imaging member including a support substrate having a two layered electrically conductive ground plane layer comprising a layer comprising zirconium over a layer comprising titanium, a hole blocking layer, and an adhesive layer. The adhesive layer of the '554 patent includes a copolyester film forming resin, and the member further includes an intermediate layer comprising a carbazole polymer, a charge generation layer comprising a perylene or a phthalocyanine, and a hole transport layer, which is substantially non-absorbing in the spectral region at which the charge generation layer generates and injects photogenerated holes. The adhesive layer of the '130 patent comprises a thermoplastic polyurethane film forming resin. The adhesive layer of the '649 patent comprises a polymer blend comprising a carbazole polymer and a film forming thermoplastic resin in contiguous contact with a hole blocking layer.

U.S. Pat. No. 5,215,839 to Robert Yu discloses a layered electrophotographic imaging member. An interface layer lies between a blocking layer and a charge generation layer, the interface layer comprising a polymer having incorporated therein filler particles of a synthetic silica or mineral particles.

U.S. Pat. No. 6,326,111 to Chambers, et al. discloses a stable charge transport layer comprising a dispersion containing polytetrafluoroethylene particles and hydrophobic silica in a polycarbonate polymer binder and at least one charge transport material.

U.S. Pat. No. 6,294,300 to Carmichael, et al. discloses a photoconductor that includes a charge transport layer coated over a charge generator layer. A hole transport molecule is intentionally added to the charge generator layer preventing migration of hole transport molecules from the charge transport layer to the charge generator layer.

U.S. Pat. No. 5,378,566 to Yu, et al. discloses an electrophotographic imaging member including a hole blocking adhesive layer. The hole blocking adhesive layer includes a polyester film forming binder having dispersed therein a particulate reaction product of metal oxide particles and a hydrolyzed reactant selected from nitrogen containing organosilanes, organotitanates and organozirconates.

U.S. Pat. No. 5,643,702 to Yu discloses an electrophotographic imaging member comprising a substrate layer, an adhesive layer comprising a thermoplastic polyurethane film forming resin, a thin vapor deposited charge generating layer

consisting essentially of a thin homogeneous vacuum sublimation deposited film of an organic photogenerating pigment, and a charge transport layer.

U.S. Pat. No. 6,379,853 to Lin, et al. discloses an imaging member including charge transporting element including two sequentially deposited charge transport layers each including a hole transport material and an optional film forming binder. A first charge transport layer exhibits a first charge carrier transit time and second charge transport layer exhibits a second charge carrier transit time.

U.S. Pat. No. 4,639,402 to Mishra et al. discloses an electrostatographic imaging member that includes a photoconductive layer comprising an organic resin binder and photoconductive particles comprising selenium coated with thin layer of a reaction product of a hydrolyzed aminosilane. Suitable binders include poly-N-vinylcarbazole and poly(hydroxyether) resin.

U.S. Pat. Nos. 5,703,487; 6,008,653; 6,119,536; and, 6,150,824 disclose methods for detecting CDS's.

U.S. Pat. No. 5,055,366 to Yu et al. discloses a protective overcoat layer containing a hole transporting carbazole polymer or polymer blend.

U.S. Pat. No. 5,149,609 to Yu et al. discloses a protective overcoat layer containing a polyester homopolymer. The homopolymer contains a hole transport compound and an aliphatic diol in its backbone. The diol is linked to the hole transport compound through an ester linkage to either a meta or para position on the hole transport compound.

## BRIEF DESCRIPTION

The present disclosure relates, in various exemplary embodiments, to an imaging member and a method of formation. In one aspect, the imaging member includes a charge transport layer that is spaced from a charge generating layer by an under-layer or barrier layer. Such an imaging member reduces charge deficiency spots.

In some embodiments, the imaging member includes an optional substrate; a charge generating layer; a charge transport layer disposed about the charge generating layer; and a barrier layer disposed between the charge generating layer and the charge transport layer. The barrier layer comprises a film forming polymeric binder material selected from a conductive binder, a non-conductive binder, and mixtures thereof, and optionally a limited concentration of a charge transport material. In specific embodiments, the barrier layer contains no charge transport material. In other specific embodiments, the barrier layer comprises only non-conductive binders; it does not contain conductive binders or charge transport material.

In other embodiments, the barrier layer may also contain a charge transport material. The charge transport material of the barrier layer is of a composition and an amount sufficient to produce a mobility of from about 10 to about 20 percent of the hole mobility of the charge transport layer. In these embodiments, the barrier layer comprises a small amount of a charge transport material, such as from about 0 to about 20 percent by weight of the barrier layer, including from about 3 percent to about 10 percent by weight of the barrier layer and about 5 percent by weight of the barrier layer.

In a further aspect, the thickness of the barrier layer is from about 1 to about 10 micrometers, including from about 2.5 to about 7.5 micrometers. In other specific embodiments, the barrier layer is from about 1 to about 2 microns thick.

In still other embodiments, the imaging member includes an optional substrate; a charge generating layer; an optional barrier layer disposed over the charge generating layer; and a

charge transport layer disposed over the optional barrier layer. The charge transport layer comprises one or more layers of charge transport molecules dispersed or dissolved in a polymer matrix, wherein the concentration of the charge transport molecules closest to the surface of the charge generating layer is reduced or at a minimum. In specific embodiments, the imaging member has first and second charge transport layers, wherein the first charge transport layer is located between the charge generating layer and the second charge transport layer and has a lower concentration of charge transport molecules than the second charge transport layer. In other specific embodiments, the first charge transport layer comprises a film forming polymeric binder material selected from a conductive binder, a non-conductive binder, and mixtures thereof, and contains no charge transport molecules.

In still further embodiments, the imaging member includes an optional substrate; a charge generating layer; a charge transport layer disposed about the charge generating layer; and a barrier layer disposed between the charge generating layer and the charge transport layer. The charge transport layer has one or more layers. In a specific embodiment, the charge transport layer has two layers. The barrier layer comprises a film forming polymeric binder material selected from a conductive binder, a non-conductive binder, and mixtures thereof, and optionally a limited concentration of a charge transport material. In specific embodiments, the barrier layer contains no charge transport material.

These and other non-limiting features or aspects of the exemplary embodiments of the present disclosure will be described with regard to the drawings and the detailed description set forth below.

#### BRIEF DESCRIPTION OF THE DRAWINGS

The following is a brief description of the drawings which is provided for the purposes of illustrating one or more of the exemplary embodiments described herein and not for the purposes of limiting the same.

FIG. 1 is a schematic cross sectional view of an exemplary flexible imaging member according to a first embodiment.

FIG. 2 is a schematic cross sectional view of an exemplary flexible imaging member according to a second embodiment.

FIG. 3 is a schematic cross sectional view of an exemplary flexible imaging member according to a third embodiment.

FIG. 4 is a graph showing the field strength versus the concentration of hole transport molecule.

#### DETAILED DESCRIPTION

The disclosure is directed, in various exemplary embodiments, to an imaging member, to a method of formation of an imaging member, and to a method of use of such an imaging member. Although the embodiments disclosed herein are applicable to electrophotographic imaging members in flexible belt configuration and rigid drum form, for reason of simplicity, the discussion below focuses on flexible belt designs.

In an aspect of an exemplary embodiment disclosed herein, there is provided an imaging member that includes a charge generating layer, a charge transport layer disposed about the charge generating layer, and an under-layer, also referred to herein as a barrier layer, disposed between the charge generating layer and the charge transport layer. The under-layer has a lower surface which is in contiguous contact with the charge generating layer, and an upper surface which is in contiguous contact with the charge transport layer. The under-layer comprises a film forming polymer binder, a film forming polymer

that functions as a charge transport carrier, or a mixture thereof. The charge transport layer is spaced apart from the charge generating layer by the under-layer and comprises one or more charge transport components, such as hole transport molecules or film forming charge transport polymers, which allow free charge photogenerated in the charge transport layer to be transported across the charge transport layer. The hole transport molecules or film forming charge transport polymers may be molecularly dispersed or dissolved in a film forming binder to form a solid solution. The under-layer is selected to inhibit the formation of charge deficient spots (CDS) in images which may otherwise occur as a result of one or more charge transport components present in the charge transport layer.

In another aspect, the charge transport component of the charge transport layer comprises an aryl amine, such as (N,N'-diphenyl-N,N'-bis[3-methylphenyl]-[1,1'-biphenyl]-4,4'-diamine)(m-TBD). The charge transport component of the charge transport layer may be molecularly dispersed in a film forming binder that has little or no inherent charge transporting capability, such as polycarbonate.

In another aspect, the under-layer comprises polyvinylcarbazole (PVK), which is an inherent hole transporting polymer. An under-layer comprising polyvinylcarbazole reduces the tendency for formation of CDS in images by m-TBD in the charge transport layer. In still another aspect, the under-layer comprises a polycarbonate, such as poly(4,4'-isopropylidene diphenyl)carbonate. In still another aspect, the hole mobility of the under-layer comprising, for example, polyvinylcarbazole and/or a polycarbonate, is less than that of the charge transport layer. The hole mobility in the under-layer may be at least 10 percent, and in one embodiment about 40 percent, of the hole mobility of the charge transport layer. For example, the hole mobility of the under-layer may be equivalent to that of a layer comprising 20 percent m-TBD dispersed in a polycarbonate binder.

To provide a further enhancement of CDS suppression, the under-layer may further comprise a dopant such as one or more of butylated hydroxytoluene (BHT), tetramethyl guanidine (TMG), triethanolamine (TEA), n-dodecylamine (DA), n-hexadecylamine (HA), 3-aminopropyltriethoxy silane, 3-aminopropyltrihydroxysilane, and their oligomers and mixtures and salts thereof. The dopant is selected to further reduce CDS and may be present in an amount of from about 20 to about 5000 ppm of the under-layer.

In one specific aspect, the under-layer includes tritylamine (TTA), 1,1-bis(4-(p-tolyl)aminophenyl) cyclohexane (TAPC); N,N'-bis(4-methylphenyl)-N,N'-bis(4-ethylphenyl)-[1,1'-(3,3'-dimethyl)biphenyl]-4,4'-diamine (Ab-16); or various combinations thereof. In another aspect, the under-layer binder includes polystyrene or other material which is less polar than the binder used in the charge transport layer. By spacing the m-TBD-containing layer from the charge generation layer with the under-layer containing one or more of these molecules, charge deficient spots are reduced.

In another aspect, the under-layer includes TAPC. TAPC has higher activation energy and, hence, lower mobility than some other charge transport molecules. Furthermore, the use of polystyrene as a binder improves the charge injection from the charge generation layer to the charge transport layer, improves charge transporting and provides a robust coating layer. This device showed good CDS reduction.

In other aspects, the concentration of the charge transport component in the charge transport layer may increase stepwise, or gradually, as for example, by an increasing concentration gradient, away from the lower surface of the charge transport layer toward the upper surface. Alternatively, the

concentration of the charge transport component in the charge transport layer may progressively increase from the region closest in proximity to the under-layer and then may decrease toward the upper region of the charge transport layer. It is to be appreciated that the charge transport layer may include one or more layers or that the composition of the charge transport layer may change gradually or stepwise.

In aspects disclosed herein, the solid solution charge transport layer may have multiple regions of different concentrations of charge transport component. The charge transport layer may comprise a solid solution of different concentrations of charge transport components, film forming polymer binders/resins and other compounds to form two or more regions.

In one aspect, the charge transport layer comprises different regions or layers of a solid solution of a film forming polymer binder containing different concentrations of charge transport component(s) wherein the layer of the largest concentration of charge transport components is spaced from the bottom surface of the charge transport layer and lower concentrations of charge transport components are at the top and bottom surfaces of the charge transport layer.

In a further embodiment, the charge transport layer can comprise multiple charge transport layers comprising a first or bottom charge transport layer comprising a solid solution of a film forming polymer binder and a charge transport component, and thereover and in contact with the first layer, a second solid solution charge transport layer or layers, the first layer being spaced from the photogenerating layer by the under-layer, the second layer having a higher concentration of charge transport component than the first layer and optionally one or more additional solid solution charge transport layers. The second layer and subsequent additional charge transport layers each can comprise the same or a different film forming polymer binder and same or different charge transport component as that of the first charge transport layer.

It has been found that the charge injection from a source such as the photogenerating layer, into the charge transport layer is influenced by the number (concentration) of charge transport molecules in the vicinity. By providing an optional under-layer and/or charge transport layer as described herein, the migration rate of charge from the charge generating layer into the charge transport layer can be suppressed and CDS spots in images generated by the imaging member can be significantly reduced. Both types of CDS spots, reduced-discharge development spots (which appear as microblack spots on white backgrounds) and charger development spots (which appear as microwhite spots on dark backgrounds), can be suppressed by lowering the concentration of the charge transport component in the under-layer adjacent to the charge generation layer. The mobility of the injected charge is also suppressed as a result of the lower concentration of charge transport component. Accordingly, the provision of a second layer that provides a higher charge mobility, for example, by incorporating a higher concentration of charge transport component, spaced from the charge generation layer, facilitates movement of the charge through the charge transport layer overall. Charge mobility can be expressed in terms of average velocity of the charge passing through a unit area per unit field of the imaging member.

The optional, additional charge transport layers in the charge transport layer may also contain a stabilizing antioxidant such as a hindered phenol. Such a phenol may be present in the top most layer of the charge transport layer in a reverse concentration gradient to that of the charge transport component. For example, while the concentration of the charge transport component increases from the first or bottom layer

(or the layer in closest proximity to the photogenerating layer) and decreases again toward the top layer in the overall charge transport layer, the concentration of the hindered phenol increases near the top surface of the charge transport layer and decreases away from it. Furthermore, in order to achieve enhanced wear resistance results, the top or uppermost layer or region of the charge transport layer may further include particles dispersions of silica, PTFE, and wax polyethylene for effective lubrication and wear life extension or be provided with an overcoat.

Advantages associated with the imaging members of the present exemplary embodiments include, for example, a reduction in charge deficient spots (CDS) in images generated with the imaging member. Additional advantages may include the avoidance or suppression of early onset of charge transport layer cracking. Such cracking or micro-cracking can be initiated by the interaction with effluent of chemical compounds, such as exposure to volatile organic compounds, like solvents, selected for the preparation of the members and corona emissions from machine charging devices. Such cracking can lead to copy print out defects and also may adversely affect functional characteristics of the imaging member.

Processes of imaging, especially xerographic imaging and printing, including digital printing, are also encompassed by the present disclosure. More specifically, the layered photoconductive imaging members can be selected for a number of different known imaging and printing processes including, for example, electrophotographic imaging processes, especially xerographic imaging and printing processes wherein charged latent images are rendered visible with toner compositions of an appropriate charge polarity. Moreover, the imaging members disclosed are useful in color xerographic applications, particularly high-speed color copying and printing processes and which members are in embodiments sensitive in the wavelength region of, for example, from about 500 to about 900 nanometers, and in particular from about 650 to about 850 nanometers, thus diode lasers can be selected as the light source.

An exemplary embodiment of a negatively charged electrophotographic imaging member of flexible belt configuration is illustrated in FIG. 1. The exemplary imaging member includes an optional support substrate 10 having an optional conductive surface layer or layers 12, an optional hole blocking layer 14, an optional adhesive layer 16, a charge generating layer 18, an under-layer (or barrier layer) 20, at least one charge transport layer 22, and optionally one or more overcoat and/or protective layer(s) 24. Other layers of the imaging member may include, for example, an optional ground strip layer 26, applied to one edge of the imaging member to promote electrical continuity with the conductive layer 12 through the hole blocking layer 14. An anti-curl back coating layer 28 may be formed on the backside of the flexible support substrate. The layers 12, 14, 16, 18, 20, 22, and 24 may be separately and sequentially deposited on the substrate 10 as solutions comprising a solvent, with each layer being dried before deposition of the next. Alternatively or additionally, the charge transport layer or the layer of the charge transport layer nearest the under-layer 20 may be applied prior to drying of the previous layer such that partial mixing at the boundaries of adjacent layers and/or leaching diffusion of one or more components from one layer into the adjacent layer(s) can occur. Under-layer 20 has a lower surface 30 that is in direct contact with the upper surface of the charge generating layer 18 and an upper surface 32 that is in direct contact with the lower surface of the charge transport layer 22.

Another exemplary embodiment is illustrated in FIG. 2. Here, the charge transport layer comprises two charge transport layers, a first (bottom) layer 22A and a second (top) layer 22B. However, compared to FIG. 1, there is no under-layer 20. In this embodiment, the first charge transport layer 22A has a lower concentration of charge transport molecules than the second charge transport layer 22B. In specific embodiments, the first charge transport layer comprises a film-forming conductive polymer, such as a carbazole, which has inherent hole transporting capability, but no charge transport molecules.

Another exemplary embodiment is illustrated in FIG. 3. Here, the charge transport layer comprises two charge transport layers, a first layer 22A and a second layer 22B.

The photoreceptor support substrate 10 may be opaque or substantially transparent, and may comprise any suitable organic or inorganic material having the requisite mechanical properties. The entire substrate can comprise the same material as that in the electrically conductive surface, or the electrically conductive surface can be merely a coating on the substrate. Any suitable electrically conductive material can be employed. Typical electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like.

The substrate 10 can also be formulated entirely of an electrically conductive material, or it can be an insulating material including inorganic or organic polymeric materials, such as, MYLAR™, a commercially available biaxially oriented polyethylene terephthalate from DuPont, MYLAR™ with a coated conductive titanium surface, otherwise a layer of an organic or inorganic material having a semiconductive surface layer, such as indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic considerations.

The substrate 10 may be flexible, being seamed or seamless for flexible photoreceptor belt fabrication or it can be rigid for use as an imaging member for plate design applications. The substrate may have a number of many different configurations, such as, for example, a plate, a drum, a scroll, an endless flexible belt, and the like. In one embodiment, the substrate is in the form of a seamed flexible belt.

The thickness of the substrate 10 depends on numerous factors, including flexibility, mechanical performance, and economic considerations. The thickness of the support substrate 10 may range from about 50 micrometers to about 3,000 micrometers; and in embodiments of flexible photoreceptor belt preparation, the thickness of substrate 10 is from about 50 micrometers to about 200 micrometers for optimum flexibility and to effect minimum induced photoreceptor surface bending stress when a photoreceptor belt is cycled around small diameter rollers in a machine belt support module, for example, 19 millimeter diameter rollers. The surface of the support substrate is cleaned prior to coating to promote greater adhesion of the deposited coating composition.

An exemplary substrate support 10 is not soluble in any of the solvents used in each coating layer solution, is optically

transparent, and is thermally stable up to a high temperature of about 150° C. A typical substrate support 10 used for imaging member fabrication has a thermal contraction coefficient ranging from about  $1 \times 10^{-5}/^{\circ}\text{C}$ . to about  $3 \times 10^{-5}/^{\circ}\text{C}$ . and a Young's Modulus of between about  $5 \times 10^5$  psi ( $3.5 \times 10^4$  Kg/cm<sup>2</sup>) and about  $7 \times 10^5$  psi ( $4.9 \times 10^4$  Kg/cm<sup>2</sup>).

The conductive layer 12 may vary in thickness depending on the optical transparency and flexibility desired for the electrophotographic imaging member. When a photoreceptor 10 flexible belt is desired, the thickness of the conductive layer 12 on the support substrate 10, for example, a titanium and/or zirconium conductive layer produced by a sputtered deposition process, typically ranges from about 20 Angstroms to about 750 Angstroms to enable adequate light transmission for proper back erase, and in embodiments from about 100 Angstroms to about 200 Angstroms for an optimum combination of electrical conductivity, flexibility, and light transmission. The conductive layer 12 may be an electrically conductive metal layer which may be formed, for example, on the substrate by any suitable coating technique, such as a vacuum depositing or sputtering technique. Typical metals suitable for use as conductive layer 12 include aluminum, zirconium, niobium, tantalum, vanadium, hafnium, titanium, nickel, stainless steel, chromium, tungsten, molybdenum, combinations thereof, and the like. Where the entire substrate is an electrically conductive metal, the outer surface thereof can perform the function of an electrically conductive layer and a separate electrical conductive layer may be omitted.

A positive charge (hole) blocking layer 14 may then 30 optionally be applied to the substrate 10 or to the layer 12, where present. Any suitable hole blocking layer capable of forming an effective barrier to holes injection from the adjacent conductive layer 12 into the photoconductive or photo-generating layer may be utilized. The charge (hole) blocking 35 layer may include polymers, such as, polyvinylbutyral, epoxy resins, polyesters, polysiloxanes, polyamides, polyurethanes, HEMA, hydroxypropyl cellulose, polyphosphazine, and the like, or may comprise nitrogen containing siloxanes or silanes, nitrogen containing titanium or zirconium compounds, such as, titanate and zirconate. Hole blocking layers having a thickness in wide range of from about 50 Angstroms (0.005 micrometers) to about 10 micrometers depending on the type of material chosen for use in a photoreceptor design. Typical hole blocking layer materials include, for example, 40 trimethoxysilyl propylene diamine, hydrolyzed trimethoxysilyl propyl ethylene diamine, N-beta-(aminoethyl) gamma-amino-propyl trimethoxy silane, isopropyl 4-aminobenzene sulfonyl, di(dodecylbenzene sulfonyl) titanate, isopropyl di(4-aminobenzoyl)isostearoyl titanate, isopropyl tri(N-ethyl-laminoethylamino)titanate, isopropyl trianthranil titanate, isopropyl tri(N,N-dimethylamino)titanate, titanium-4-amino benzene sulfonate oxyacetate, titanium 4-aminobenzoate isostearate oxyacetate,  $[\text{H}_2\text{N}(\text{CH}_2)_4]\text{CH}_3\text{Si}(\text{OCH}_3)_2$ , (gammaaminobutyl)-methyl diethoxysilane, and  $[\text{H}_2\text{N}(\text{CH}_2)_3]\text{CH}_3\text{Si}(\text{OCH}_3)_2$ , (gammaaminopropyl)-methyl diethoxysilane, and combinations thereof, as disclosed in U.S. Pat. Nos. 4,338,387, 4,286,033 and 4,291,110, incorporated herein by reference in their entireties. Other suitable charge blocking layer polymer compositions are also 50 described in U.S. Pat. No. 5,244,762 which is incorporated herein by reference in its entirety. These include vinyl hydroxyl ester and vinyl hydroxy amide polymers wherein the hydroxyl groups have been partially modified to benzoate and acetate esters which modified polymers are then blended 55 with other unmodified vinyl hydroxyl ester and amide unmodified polymers. An example of such a blend is a 30 mole percent benzoate ester of poly (2-hydroxyethyl meth-

## 11

acrylate) blended with the parent polymer poly (2-hydroxyethyl methacrylate). Still other suitable charge blocking layer polymer compositions are described in U.S. Pat. No. 4,988,597, which is incorporated herein by reference in its entirety. These include polymers containing an alkyl acrylamidoglycolate alkyl ether repeat unit. An example of such an alkyl acrylamidoglycolate alkyl ether containing polymer is the copolymer poly(methyl acrylamidoglycolate methyl ether-co-2-hydroxyethyl methacrylate). The disclosures of these U.S. Patents are incorporated herein by reference in their entireties.

The blocking layer 14 is continuous and may have a thickness of less than about 10 micrometers because greater thicknesses may lead to undesirably high residual voltage. In aspects of the exemplary embodiment, a blocking layer of from about 0.005 micrometers to about 2 micrometers facilitates charge neutralization after the exposure step and optimum electrical performance is achieved. The blocking layer may be applied by any suitable conventional technique, such as, spraying, dip coating, draw bar coating, gravure coating, silk screening, air knife coating, reverse roll coating, vacuum deposition, chemical treatment, and the like. For convenience in obtaining thin layers, the blocking layer may be applied in the form of a dilute solution, with the solvent being removed after deposition of the coating by conventional techniques, such as, by vacuum, heating, and the like. Generally, a weight ratio of blocking layer material and solvent of between about 0.05:100 to about 5:100 is satisfactory for spray coating.

The optional adhesive layer 16 may be applied to the hole blocking layer 14. Any suitable adhesive layer may be utilized. One well known adhesive layer includes a linear saturated copolyester reaction product of four diacids and ethylene glycol. This linear saturated copolyester consists of alternating monomer units of ethylene glycol and four randomly sequenced diacids in the above indicated ratio and has a weight average molecular weight of about 70,000. If desired, the adhesive layer may include a copolyester resin. The adhesive layer is applied directly to the hole blocking layer. Thus, the adhesive layer in embodiments is in direct contiguous contact with both the underlying hole blocking layer and the overlying charge generating layer to enhance adhesion bonding to provide linkage. In embodiments, the adhesive layer is continuous.

Any suitable solvent or solvent mixtures may be employed to form a coating solution of the polyester. Typical solvents include tetrahydrofuran, toluene, methylene chloride, cyclohexanone, and the like, and mixtures thereof. Any other suitable and conventional technique may be used to mix and thereafter apply the adhesive layer coating mixture to the hole blocking layer. Typical application techniques include spraying, dip coating, roll coating, wire wound rod coating, and the like. Drying of the deposited wet coating may be effected by any suitable conventional process, such as oven drying, infrared radiation drying, air drying, and the like.

The adhesive layer 16 may have a thickness of from about 0.01 micrometers to about 900 micrometers after drying. In embodiments, the dried thickness is from about 200 micrometers and about 900 micrometers, although thicknesses of from about 0.03 micrometers to about 1 micrometer are satisfactory for some applications. At thicknesses of less than about 0.01 micrometers, the adhesion between the charge generating layer and the blocking layer is poor and delamination can occur when the photoreceptor belt is transported over small diameter supports such as rollers and curved skid plates.

The charge generating layer 18 may thereafter be applied to the blocking layer 14 or the adhesive layer 16, if one is

## 12

employed. Any suitable charge generating binder layer 18 including a photogenerating/photoconductive material, which may be in the form of particles and dispersed in a film forming binder, such as an inactive resin, may be utilized. Examples of photogenerating materials include, for example, inorganic photoconductive materials such as amorphous selenium, trigonal selenium, and selenium alloys selected from the group consisting of selenium-tellurium, selenium-tellurium-arsenic, selenium arsenide and mixtures thereof, and organic photoconductive materials including various phthalocyanine pigment such as the X-form of metal free phthalocyanine, metal phthalocyanines such as vanadyl phthalocyanine and copper phthalocyanine, quinacridones, dibromo anthanthrone pigments, benzimidazole perylene, substituted 2,4-diamino-triazines, polynuclear aromatic quinones, and the like dispersed in a film forming polymeric binder. Selenium, selenium alloy, benzimidazole perylene, and the like and mixtures thereof may be formed as a continuous, homogeneous photogenerating layer. Benzimidazole perylene compositions are well known and described, for example, in U.S. Pat. No. 4,587,189, the entire disclosure thereof being incorporated herein by reference. Multi-photogenerating layer compositions may be utilized where a photoconductive layer enhances or reduces the properties of the photogenerating layer. Other suitable photogenerating materials known in the art may also be utilized, if desired. The photogenerating materials selected should be sensitive to activating radiation having a wavelength from about 400 nm to about 850 nm and about 700 nm to about 850 nm during the imagewise radiation exposure step in an electrophotographic imaging process to form an electrostatic latent image.

Any suitable inactive resin materials may be employed in the photogenerating layer 18, including those described, for example, in U.S. Pat. No. 3,121,006, the entire disclosure thereof being incorporated herein by reference. Typical organic resinous binders include thermoplastic and thermosetting resins such as one or more of polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like.

The photogenerating material can be present in the resinous binder composition in various amounts. Generally, from about 5 percent by volume to about 90 percent by volume of the photogenerating material is dispersed in about 10 percent by volume to about 95 percent by volume of the resinous binder, and more specifically from about 30 percent by volume to about 50 percent by volume of the photogenerating material is dispersed in about 50 percent by volume to about 70 percent by volume of the resinous binder composition.

The photogenerating layer 18 containing the photogenerating material and the resinous binder material generally ranges in thickness of from about 0.1 micrometer to about 5 micrometer for example, from about 0.3 micrometers to about 3 micrometers when dry. The photogenerating layer

## 13

thickness is generally related to binder content. Higher binder content compositions generally employ thicker layers for photogeneration.

The next layers applied over the charge generating layer **18** include under-layer **20** and charge transport layer **22**. The under-layer **20**, which is also referred to herein as a barrier layer, is applied over the charge generating layer **18**, and charge transport layer **22** is then applied over the barrier or under-layer. Thus, barrier or under-layer **20** spaces the charge transport layer **22** away from charge generating layer **18**.

In conventional imaging members, the charge transport layer is applied directly over the charge generating layer, and there is typically a relatively large concentration of charge transport molecules along the interface between the charge generating layer and the charge transport layer. The presence of charge transport molecules at this interface causes or results in charge deficient spots (CDS) defects in print-out copies. By spacing the charge transport layer away from the charge generating layer with a barrier layer intermediate the charge transport layer and the charge generating layer, the concentration of charge transport molecules near the surface of the charge generating layer can be reduced or eliminated, which will reduce or eliminate charge deficient spots.

Barrier or under-layer **20** consists essentially of a film forming polymeric binder material. The polymeric binder material may be a conductive polymer binder, a non-conductive polymer binder, or mixtures of conductive and non-conductive polymer binder materials. As will be discussed below, the barrier layer may also include a relatively small concentration of charged transport molecules.

The barrier layer may also include or be formed from a non-conductive or inactive polymer binder. Suitable non-conductive polymer binders include those that are typically used in other layers of an imaging member such as the photogenerating layer or the charge transport layer. Suitable non-conductive binders include, but are not limited to, polycarbonate resin, polyester, polyarylate, polyacrylate, polyether, polysulfone, polyvinyl butyral, polyvinyl formals, and combinations thereof. Exemplary polycarbonates include poly(4-4'-isopropylidene diphenyl carbonate), poly(4,4'-diphenyl-1-1'-cyclohexene carbonate), and the like. An exemplary polycarbonate is a Makrolon™ binder, which is available from Bayer AG and comprises poly(4-4'-isopropylidene diphenyl) carbonate having a weight average molecular weight of about 120,000.

The barrier or under-layer consists predominantly of polymeric binder. The barrier or under-layer may include from about 90 to about 100 percent by weight of polymeric binder material. The polymeric binder may include a conductive polymer binder, non-conductive polymer binder, and mixtures of conductive and non-conductive binders. In one embodiment, for example, the barrier layer consists essentially of about 100 percent by weight of a conductive polymer binder. In another embodiment, the barrier layer consists essentially of about 100 percent by weight of a non-conductive polymer binder. It will be appreciated that an under-layer consisting essentially of either a conductive binder or a non-conductive binder may include mixtures of conductive binders or mixtures of non-conductive binders. In a composition that is a mixture of a conductive and non-conductive polymer binder, the conductive polymer binder may be present in an

## 14

amount of from about 1 to about 99 percent by weight, and the non-conductive binder may be present in an amount of 99 to about 1 percent by weight. In another embodiment, a mixture of conductive and non-conductive polymer binders may comprise from about 30 to about 70 percent by weight of a conductive polymer binder, and from about 70 to about 30 percent by weight of a non-conductive polymer. In still another embodiment, a mixture of conductive and non-conductive polymer binder may comprise from about 40 to about 60 percent by weight of a conductive polymer binder, and from about 60 to about 40 percent by weight of a non-conductive polymer binder. These embodiments of barrier layers do not contain charge transport molecules, but may contain other additives. The basic characteristic is that charge transport molecules are not present at the interface between the barrier layer and the charge generating layer.

Charge transport molecules or materials in the barrier or under-layer may be present by design or by the nature of forming the charge transport layer over the barrier layer. Thus in one embodiment, the charge transport material may be included in a composition with a conductive and/or non-conductive binder that is used to form the barrier or under-layer. In another embodiment, the charge transport material may be present in the barrier or under-layer as a result of diffusion of charge transport material into the barrier layer from the composition used to form the charge transport layer as the charge transport layer is applied over the barrier layer. Regardless of how charge transport material is present, if it all, in the barrier layer, the concentration of charge transport material that is present along the interface between the charge generating layer and the barrier layer is reduced or eliminated compared to conventional imaging members where the charge transport layer is applied directly over the charge generating layer.

The barrier layer may have from about 0 to about 20 percent by weight of a charge transport material. In one embodiment, the barrier or under-layer includes a charge transport material in an amount from about greater than 0 percent by weight to about 10 percent by weight. In another embodiment, the barrier layer includes from about 3 to about 10 percent by weight of a charge transport material. In another embodiment, the barrier layer may include about 5 percent by weight of a charge transport material. In another embodiment, the barrier layer contains no charge transport material. The charge transport material present in the barrier layer is not limited in any manner, and may be selected from any material or molecule known in the art or later discovered to be capable of acting as a charge transport molecule as is understood in the art.

The barrier or under-layer may have any thickness as desired for a particular purpose or intended use. As the thickness of the barrier layer increases, charge deficiency spots may be reduced relative to thinner layers. In thicker barrier layers, while charge transport material from the charge transport layer above the barrier layer will likely diffuse into the barrier layer, the depth of penetration is not as great as compared to barrier layers of smaller thickness. Consequently, there is a smaller concentration of charge transport material near the lower surface of the barrier layer. In one embodiment, the barrier layer has a thickness of from about 1 to about 10 micrometers. In another embodiment, the barrier layer has a thickness of from about 2.5 to about 7.5 micrometers. In another embodiment, the barrier layer has a thickness of from about 1 to about 2 micrometers.

15

Examples of suitable charge transport materials that may be included in the barrier or under-layer and the charge transport layer include those described in co-pending application Ser. Nos. 10/736,864, 10/744,369, and 10/320,808, all of which are incorporated herein by reference in their entirety. Other exemplary charge transporting materials include aromatic diamines, such as aryl diamines. Exemplary aromatic diamines include, but are not limited to, N,N'-diphenyl-N,N'-bis(alkylphenyl)-1,1'-biphenyl-4,4'-diamines, such as m-TBD, which has the formula N,N'-diphenyl-N,N'-bis[3-methylphenyl]-[1,1'-biphenyl]-4,4'-diamine; p-TBD, which has the formula N,N'-diphenyl-N,N'-bis[4-methylphenyl]-[1,1'-biphenyl]-4,4'-diamine; N,N'-diphenyl-N,N'-bis(chlorophenyl)-1,1'-biphenyl-4,4'-diamine; N,N'-bis(4-ethylphenyl)-1,1'-(3,3'-dimethylbiphenyl)-4,4'-diamine (Ae-16); N,N'-bis(4-methoxy-2-methylphenyl)-N,N'-diphenyl-[1,1'-biphenyl]-4,4'-diamine and combinations thereof. Another suitable charge transport material is 1,1-bis(di-4-tolylaminophenyl)cyclohexane (TAPC). Other exemplary charge transport materials include arylamines such as tri(4-methylphenyl)amine, N,N-di(3,4-dimethyl)phenyl, N-(4-biphenyl)amine, and the like.

In the imaging member according to FIG. 2, the under-layer is not present. Instead, the charge transport layer comprises a first charge transport layer 22A and a second charge transport layer 22B. The first charge transport layer comprises a film forming polymer having inherent hole transporting capability. The second charge transport layer comprises a polymer binder and a charge transport material. In some embodiments, the first charge transport layer 22A is required to have an intrinsic hole transporting mobility at least equivalent to that of a charge transport layer consisting of 75 percent by weight of Makrolon™ and 25 percent by weight of m-TBD. The first charge transport layer 22A must be optically clear to allow effective imaging formation in the charge generation layer 18 during electrophotographic imaging process. In other embodiments, the first charge transport layer is a mixture of hole transporting polymers, with no charge transport material included.

One example of a conductive, hole-transporting polymer binder suitable for the optional barrier layer and/or for the first charge transport layer is a carbazole polymer. In one embodiment a polycarbazole may be a material of the formula



wherein R<sub>1</sub> is selected from



wherein n is the degree of polymerization; and R<sub>2-5</sub> are independently selected from H, alkyl, substituted alkyl, alkoxy,

16

and the like and combinations thereof. In one embodiment, the conductive polymer binder includes polyvinyl carbazole, which has the formula



In other embodiments, the carbazole polymer is one of the following formulas:



A second hole transporting polymer suitable for the optional barrier layer and/or the first charge transport layer is a polyester homopolymer having an ester linkage to either the meta or para position of a selected aryl diamine hole transport compound. Exemplary aryl diamines include N,N'-diphenyl-N,N'-bis(alkylphenyl)-1,1'-biphenyl-4,4'-diamines, such as m-TBD, which has the formula N,N'-diphenyl-N,N'-bis[3-methylphenyl]-[1,1'-biphenyl]-4,4'-diamine as well as p-TBD, which has the formula N,N'-diphenyl-N,N'-bis[4-methylphenyl]-[1,1'-biphenyl]-4,4'-diamine; N,N'-diphenyl-N,N'-bis(chlorophenyl)-1,1'-biphenyl-4,4'-diamine; N,N'-bis(4-ethylphenyl)-1,1'-(3,3'-dimethylbiphenyl)-4,4'-diamine (Ae-16); and N,N'-bis(4-methoxy-2-methylphenyl)-N,N'-diphenyl-[1,1'-biphenyl]-4,4'-diamine. The molecular structure of the polyester homopolymer having the ester in a meta linkage is shown below:



The molecular structure of the polyester homopolymer having the ester in a para linkage is shown below:



In both of these embodiments, x is from 2 to 20 and m is the degree of polymerization.

A third set of hole transport polymers suitable for the optional barrier layer and/or the first charge transport layer are organopolyphosphazenes having the following structures:



wherein R is selected from a pendant group having intrinsic hole transport capability and y is the degree of polymerization. For example, R may be a linear chain containing an aryl diamine such as one of the charge transport molecules described above.

A hole transporting polymer suitable for the optional barrier layer and/or the first charge transport layer may also be selected from the group consisting of a hole transport compound-urethane copolymer, a fluorine-based pendant active moiety of a polyester, a fluorine-based active moiety polycarbonate, and a fluorine based active moiety polyurethane.

Although the first charge transport layer 22A of present disclosure is formed from any one of these inherent hole transporting polymers, nonetheless it may also be alternatively formulated to give a blend by mixing of two or more of the hole transporting polymers; and again, the first charge

35 transport layer thus formed must be optically clear to allow effective imaging formation in the charge generation layer 18 during electrophotographic imaging process.

The two charge transport layers together have a thickness ranging from about 20 to about 50 micrometers. The thickness of the first charge transport layer 22A of this disclosure 40 is between about 120 percent and about 40 percent of the thickness of the second charge transport layer 22B. In specific embodiments, the thickness of the first charge transport layer is from about 100 percent to about 50 percent the thickness of the second charge transport layer. The thickness of the first 45 layer is usually equal to or slightly less than that of the second layer. In general, the ratio of the thickness of the charge transport layer 22 to the charge generator layer 18 is maintained from about 2:1 to about 200:1 and in some instances as great as about 400:1.

50 In one particular embodiment, the second charge transport layer 22B is formulated as a binary solid solution comprising between about 45 and 75 percent by weight of hole transport compound in a non conductive polymer binder, based on the 55 total weight of the layer 22B. The first charge transport layer 22A comprises a hole transporting polymer but no charge transport material. This construction suppresses or eliminates hole transport compound migration/diffusion to the lower surface 34 during application of the second charge transport 60 layer 22B. Elimination/suppression of the presence of hole transport compound at the lower surface 34 has been experimentally determined to be the key to reducing the propensity of CDS defects in copy print-outs. In one embodiment, the hole transport compound and polymer binder used in the 65 second charge transport layer 22B are (N,N'-diphenyl-N,N'-bis[3-methylphenyl]-[1,1'-biphenyl]-4,4'-diamine and Makrolon<sup>TM</sup>.

In additional embodiments, the charge transport layer may comprise multiple sublayers. For example, in one there may be from 2 to about 15 sublayers, such as two, three, five, six, or eight sublayers. In these multiple sublayers, the content of charge transport compound in each sublayer increases in order from the bottom sublayer adjacent to the charge generating layer up to the top outermost sublayer, where the content is based on the amount of charge transport compound in each sublayer. In alternative embodiments, the content of charge transport compound in each sublayer may be decreased in order from the bottom sublayer adjacent to the charge generating layer up to the top outermost sublayer, where the content is based on the amount of charge transport compound in each sublayer, to give the top layer mechanical functioning life enhancement. However, the total amount of charge transport compound, in either case, is still maintained from about 45 to about 75 percent by weight based on the total weight of the sublayers. In additional embodiments, LCM control agents are also present in the sublayers and their concentration decreases in order from the top outermost sublayer down to the bottommost sublayer. Wear enhancement particle dispersions, if used, are added only to the outermost exposed sublayer.

The charge transport layer 22B may be formed by depositing a single layer or sequential deposition of multiple sublayers. In one embodied process, the sublayers are not dried or are only partially dried prior to application of the subsequent sub-layer. As a result, partial mixing and/or diffusion of the charge transport component at the boundaries between the two sublayers, and a more gradual variation or a concentration gradient continuum compared to stepwise variation, in concentration of the charge transport component is achieved. This partial mixing and/or diffusion occurs only between the two sublayers; the charge transport component will not diffuse into a third sublayer. For example, solutions of different concentrations can be deposited via separate slots in a slotted extrusion die to form sublayers on the barrier layer or the charge generating layer.

In embodiments comprising three sublayers, the third sublayer has a lower concentration of the charge transport component than the second sublayer. The charge mobility in the third sublayer may thus be lower than in the second sublayer. The concentration of the charge transport component in the third sublayer can be from about 1 percent to about 95 percent of the concentration of the charge transport component in the second sublayer (or from about 1 percent to about 95 percent of the highest concentration in the second sublayer, where the concentration varies in the second sublayer). In one embodiment the charge transport component concentration in the third sublayer is at least about 5 percent that of the second sublayer, in another embodiment, at least about 20 percent, and in yet another embodiment, at least 30 percent. The charge transport component concentration in the third sublayer can be from about 50 percent to about 300 percent of the concentration in the first sublayer. The concentration of the charge transport component in the charge transport layer, in one embodiment, increases from the first sublayer adjacent to the barrier layer 20 to the second sublayer, then decreases in the third sublayer, the concentration being determined for each individual sublayer. The third sublayer may comprise, for example, from about 5 to about 50 weight percent of charge transport component. In one embodiment, it comprises from about 5 to about 45 weight percent of charge transport component.

In another embodiment according to FIG. 3, the imaging member has a charge generating layer 18, a barrier layer 20, and a first charge transport layer 22A and a second charge

transport layer 22B, both formed to comprise a charge transport component and a polymer binder. The first charge transport layer 22A has a lower concentration of charge transport component than the second layer 22B. The first layer may comprise from about 5 to about 40 weight percent of charge transport component, based on the weight of the first layer. In specific embodiments, it comprises from about 10 to about 35 weight percent of charge transport component. The second layer may comprise from about 30 to about 90 weight percent of charge transport component, based on the weight of the second layer. In more specific embodiments, it comprises from about 35 to about 50 weight percent of charge transport component. Because of a greater concentration of charge transport component, the charge mobility in the second layer is higher than in the first layer. Though at low concentration, the effects of the low concentration of the charge transport component in the first layer on the charge mobility can be offset by making the first layer of a lower thickness than second layer.

The outermost top charge transport layer of the imaging member may also include antioxidants, leveling agents, surfactants, wear resistant fillers such as dispersion of polytetrafluoroethylene (PTFE) particles and silica particles, light shock resisting or reducing agents, and the like, to impart further desired photo-electrical, mechanical, and copy print-out quality properties, particularly if no overcoat layer is used.

Antioxidant, such as a hindered phenol, may be added to improve electrical stability and minimize LCM. Exemplary hindered phenols include octadecyl-3,5-di-tert-butyl-4-hydroxyhydrocinnamate, available as Irganox I-1010 from Ciba Specialty Chemicals. The hindered phenol may be present at about 10 weight percent in the top sublayer, based on the weight of the top sublayer. The hindered phenol concentration may also vary among all of the charge transport sublayers to create a concentration gradient opposite that of the charge transport component.

A nanoparticle dispersion, such as silica, metal oxides, Acumist™ (waxy polyethylene particles), PTFE, and the like, may be used to enhance lubricity and wear resistance. The particle dispersion may be present at about 10 weight percent in the top sublayer, based on the weight of the top sublayer, to provide optimum wear resistance without causing a deleterious impact on the electrical properties of the fabricated imaging member.

The charge transport layer 22, for a negatively charged imaging member of FIG. 1, is applied over the under-layer 20 and may include any suitable transparent organic polymer or non-polymeric material capable of supporting the injection of photogenerated holes from the charge generating layer 18 via the under-layer 20 and capable of allowing the transport of these holes through the charge transport layer to selectively discharge the surface charge on the imaging member surface. In one embodiment, the charge transport layer 22 not only serves to transport holes, but also protects the charge generating layer 18 from abrasion or chemical attack and may therefore extend the service life of the imaging member. The charge transport layer may be a single layer or multi-layer configuration according to FIGS. 2 and 3. Multi-layer configurations comprise two or more charge transport layers. Any individual layers or sublayers of the overall charge transport layer are normally transparent in a wavelength region in which the electrophotographic imaging member is to be used when exposure is effected therethrough to ensure that most of the incident radiation is utilized by the charge generating layer 18. Each charge transport layer in a multi-layered charge transport layer configuration should exhibit excellent

optical transparency with negligible light absorption and neither charge generation nor discharge if any, when exposed to a wavelength of light useful in xerography, e.g., 4000 to 9000 Angstroms. When the photoreceptor is prepared with the use of a transparent substrate **10** and also a transparent conductive layer **12**, imagewise exposure or erase may be accomplished through the substrate **10** with all light passing through the back side of the substrate. In this case, the materials of the charge transport layer's individual layers or sub-layers need not transmit light in the wavelength region of use if the charge generating layer **18** is sandwiched between the substrate and the charge transport layer **22**. The charge transport layer **22** in conjunction with the charge generating layer **18** is an insulator to the extent that an electrostatic charge placed on the charge transport layer is not conducted in the absence of illumination. The charge transport layer **22** and any intermediate and top charge transport layers should trap minimal charges as the case may be passing through it. Charge transport layer materials are well known in the art.

The charge transport layer **22** may include any suitable charge transport component or activating compound useful as an additive molecularly dispersed in an electrically inactive polymeric material to form a solid solution and thereby making this material electrically active. The charge transport component typically comprises small molecules of an organic compound that cooperates to transport charge between molecules and ultimately to the surface of the charge transport layer.

Although the film forming polymer binder used in the multiples of sublayers may be different for different charge transport layers, in one embodiment, an identical polymer binder is used throughout all the multiples of the charge transport layer which tends to provide improved interfacial adhesion bonding between any individual charge transport layers.

Any suitable inactive resin binder soluble in methylene chloride, chlorobenzene, or other suitable solvent may be employed in the charge transport layer. Exemplary binders include polyesters, polyvinyl butyral, polycarbonates, polystyrene, polyvinyl formals, and combinations thereof. The polymer binder used for the charge transport layers may be, for example, selected from the group consisting of polycarbonates, polyester, polyarylate, polyacrylate, polyether, polysulfone, combinations thereof, and the like. Exemplary polycarbonates include poly(4,4'-isopropylidene diphenyl carbonate), poly(4,4'-diphenyl-1,1'-cyclohexene carbonate), and combinations thereof. The molecular weight of the binder can be for example, from about 20,000 to about 1,500,000. One exemplary binder of this type is a Makrolon<sup>TM</sup> binder, which is available from Bayer AG and comprises poly(4,4'-isopropylidene diphenyl) carbonate having a weight average molecular weight of about 120,000.

Exemplary charge transport components include those described in above-mentioned co-pending application Ser. Nos. 10/736,864, 10/744,369, and 10/320,808, incorporated herein by reference, which may be used singly or in combination for individual charge transport layers in a charge transport having a multi-layer configuration. Exemplary charge transporting components include aromatic diamines, such as aryl diamines. Exemplary diphenyl diamines suited for use as the charge component, singly or in combination, are represented by the molecular Formula 1 below:



wherein X is independently selected from the group consisting of alkyl, hydroxy, and halogen. Typically, the halogen is a chloride. Where X is alkyl, X can comprise from 1 to about 10 carbon atoms, e.g., from 1 to 5 carbon atoms, such as methyl, ethyl, propyl, butyl, and the like. Exemplary aromatic diamines of this type include N,N'-diphenyl-N,N'-bis(alkylphenyl)-1,1'-biphenyl-4,4'-diamines, such as m-TBD, which has the formula N,N'-diphenyl-N,N'-bis[3-methylphenyl]-[1,1'-biphenyl]-4,4'-diamine; p-TBD, which has the formula N,N'-diphenyl-N,N'-bis[4-methylphenyl]-[1,1'-biphenyl]-4,4'-diamine; N,N'-diphenyl-N,N'-bis(chlorophenyl)-1,1'-biphenyl-4,4'-diamine; N,N'-bis(4-ethylphenyl)-1,1'-(3,3'-dimethylbiphenyl)-4,4'-diamine (Ae-16), and combinations thereof.

In one specific embodiment, the charge transport layer **22** is a solid solution including a charge transport component, such as m-TBD, molecularly dissolved in a polycarbonate binder, the binder being either a poly(4,4'-isopropylidene diphenyl carbonate) or a poly(4,4'-diphenyl-1,1'-cyclohexane carbonate). The charge transport layer may have a Young's Modulus in the range of from about  $2.5 \times 10^5$  psi ( $1.7 \times 10^4$  Kg/cm<sup>2</sup>) to about  $4.5 \times 10^5$  psi ( $3.2 \times 10^4$  Kg/cm<sup>2</sup>) and a thermal contraction coefficient of between about  $6 \times 10^{-5}/^{\circ}$  C. and about  $8 \times 10^{-5}/^{\circ}$  C.

Other layers such as conventional ground strip layer **26** including, for example, conductive particles dispersed in a film forming binder may be applied to one edge of the imaging member to promote electrical continuity with the conductive layer **12** through the hole blocking layer **14**, and adhesive layer **16**. Ground strip layer **26** may include any suitable film forming polymer binder and electrically conductive particles. Typical ground strip materials include those enumerated in U.S. Pat. No. 4,664,995, the entire disclosure of which is incorporated by reference herein. The ground strip layer **26** may have a thickness from about 7 micrometers to about 42 micrometers, for example, from about 14 micrometers to about 23 micrometers. Optionally, an overcoat layer **24**, if desired, may also be utilized to provide imaging member surface protection as well as improve resistance to abrasion and scratching.

Where an overcoat layer **24** is employed, it may comprise a similar resin used for the charge transport layer or a different resin and be from about 1 to about 2 microns in thickness.

Since the charge transport layer **22** or the multiples of sublayers can have a substantial thermal contraction mismatch compared to that of the substrate support **10**, the prepared flexible electrophotographic imaging member may exhibit spontaneous upward curling due to the result of larger dimensional contraction in the charge transport layer **20** than the substrate support **10**, as the imaging member cools down to room ambient temperature after the heating/drying processes of the applied wet charge transport layer coating. An anti-curl back coating **28** can be applied to the back side of the

substrate support **10** (which is the side opposite the side bearing the electrically active coating layers) in order to render flatness.

The anti-curl back coating **28** may include any suitable organic or inorganic film forming polymers that are electrically insulating or slightly semi-conductive. The anti-curl back coating **28** used has a thermal contraction coefficient value substantially greater than that of the substrate support **10** used in the imaging member over a temperature range employed during imaging member fabrication layer coating and drying processes (typically between about 20° C. and about 130° C.). To yield the designed imaging member flatness outcome, the applied anti-curl back coating has a thermal contraction coefficient of at least about 1.5 times greater than that of the substrate support to be considered satisfactory; that is a value of at least approximately  $1 \times 10^{-5}/^{\circ}\text{C.}$  greater than the substrate support, which typically has a substrate support thermal contraction coefficient of about  $2 \times 10^{-5}/^{\circ}\text{C.}$  However, an anti-curl back coating with a thermal contraction coefficient at least about 2 times greater, equivalent to about  $2 \times 10^{-5}/^{\circ}\text{C.}$  greater than that of the substrate support is appropriate to yield an effective anti-curling result. The applied anti-curl back coating **28** can be a film forming thermoplastic polymer, being optically transparent, with a Young's Modulus of at least about  $2 \times 10^5$  psi ( $1.4 \times 10^4$  Kg/cm<sup>2</sup>), bonded to the substrate support to give at least about 15 gms/cm of 180° peel strength. The anti-curl back coating **28** may be from about 7 to about 20 weight percent based on the total weight of the imaging member, which may correspond to from about 7 to about 20 micrometers in dry coating thickness. The selected anti-curl back coating is readily applied by dissolving a suitable film forming polymer in any convenient organic solvent.

Exemplary film forming thermoplastic polymers suitable for use in the anti-curl back coating include polycarbonates, polystyrenes, polyesters, polyamides, polyurethanes, polyarylethers, polyarylsulfones, polyarylate, polybutadienes, polysulfones, polyethersulfones, polyethylenes, polypropylenes, polyimides, polymethylpentenes, polyphenylene sulfides, polyvinyl acetate, polysiloxanes, polyacrylates, polyvinyl acetals, polyamides, polyimides, amino resins, phenylene oxide resins, terephthalic acid resins, phenoxy resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride-vinylchloride copolymers, vinylacetate-vinylidenechloride copolymers, styrene-alkyd resins, combinations thereof, and the like. These polymers may be block, random or alternating copolymers. Molecular weights can vary from about 20,000 to about 150,000. Suitable polycarbonates include bisphenol A polycarbonate materials, such as poly(4,4'-isopropylidene-diphenylene carbonate) having a molecular weight of from about 35,000 to about 40,000, available as Lexan 145<sup>TM</sup> from General Electric Company and poly(4,4'-isopropylidene-diphenylene carbonate) having a molecular weight of from about 40,000 to about 45,000, available as Lexan 141<sup>TM</sup> also from the General Electric Company. A bisphenol A polycarbonate resin having a molecular weight of from about 50,000 to about 120,000, is available as Makrolon<sup>TM</sup> from Farbenfabriken Bayer A.G. A lower molecular weight bisphenol A polycarbonate resin having a molecular weight of from about 20,000 to about 50,000 is available as Merlon<sup>TM</sup> from Mobay Chemical Company. Another suitable polycarbonate is poly(4,4-diphenyl-1,1'-cyclohexene carbonate), which is a film forming thermoplastic polymer comprising a structurally modified from bisphenol A

polycarbonate which is commercially available from Mitsubishi Chemicals. All of these polycarbonates have a Tg of between about 145° C. and about 165° C. and with a thermal contraction coefficient ranging from about  $6.0 \times 10^{-5}/^{\circ}\text{C.}$  to about  $7.0 \times 10^{-5}/^{\circ}\text{C.}$

Furthermore, suitable film forming thermoplastic polymers for the anti-curl back coating **28**, if desired, may include the same binder polymers used in the charge transport layer **22**. The anti-curl back coating formulation may include a small quantity of a saturated copolyester adhesion promoter to enhance its adhesion bond strength to the substrate support. Typical copolyester adhesion promoters are Vitel<sup>TM</sup> polyesters from Goodyear Rubber and Tire Company, Mor-Ester<sup>TM</sup> polyesters from Morton Chemicals, Eastar PETG<sup>TM</sup> polyesters from Eastman Chemicals, and the like. To impart optimum wear resistance as well as maintaining the coating layer optical clarity, the anti-curl layer may further incorporate in its material matrix, about 5 to about 30 weight percent filler dispersion of silica particles, Teflon particles, PVF2 particles, stearate particles, aluminum oxide particles, titanium dioxide particles or a particle blend dispersion of Teflon<sup>TM</sup> and any of these inorganic particles. Suitable particles used for dispersion in the anti-curl back coating include particles having a size of between about 0.05 and about 0.22 micrometers, and more specifically between about 0.18 and about 0.20 micrometers.

In one embodiment, the anti-curl back coating **28** is optically transparent. The term optically transparent is defined herein as the capability of the anti-curl back coating to transmit at least about 98 percent of an incident light energy through the coating. The anti-curl back coating of this embodiment includes a film forming thermoplastic polymer and may have a glass transition temperature (Tg) value of at least about 75° C., a thermal contraction coefficient value of at least about 1.5 times greater than the thermal contraction coefficient value of the substrate support, a Young's Modulus of at least about  $2 \times 10^5$  p.s.i., and adheres well over the supporting substrate to give a 180° peel strength value of at least about 15 grams/cm.

The multilayered, flexible electrophotographic imaging member web stocks having an under-layer and charge transport layer fabricated in accordance with the embodiments of the present disclosure as described herein may be cut into rectangular sheets. The opposite end pair of each cut sheet is then brought to overlap and joined by any suitable means, such as ultrasonic welding, gluing, taping, stapling, or pressure and heat fusing to form a continuous imaging member seamed belt, sleeve, or cylinder. The prepared flexible imaging belt may thereafter be employed in any suitable and conventional electrophotographic imaging process which utilizes uniform charging prior to imagewise exposure to activating electromagnetic radiation. When the imaging surface of an electrophotographic member is uniformly charged with an electrostatic charge and imagewise exposed to activating electromagnetic radiation, conventional positive or reversal development techniques may be employed to form a marking material image on the imaging surface of the electrophotographic imaging member. Thus, by applying a suitable electrical bias and selecting toner having the appropriate polarity of electrical charge, a toner image is formed in the charged areas or discharged areas on the imaging surface of the electrophotographic imaging member. For example, for positive development, charged toner particles are attracted to the oppositely charged electrostatic areas of the imaging surface and for reversal development, charged toner particles are attracted to the discharged areas of the imaging surface.

The development will further be illustrated in the following non-limiting working examples. These examples are intended to be illustrative only and the disclosure is not intended to be limited to the materials, conditions, process parameters and the like recited herein. All proportions are by weight unless otherwise indicated.

## REFERENCE EXAMPLE I

In these examples, reference imaging members, control imaging members, and imaging members of the present disclosure were prepared for comparison and assessment of each respective potential effectiveness of CDS suppression. Six electrophotographic imaging members were prepared by providing a 0.02 micrometer thick titanium layer coated on a substrate web of a biaxially oriented polyethylene terephthalate substrate having a thickness of 3.0 mils (89 micrometers). The titanized substrate was extrusion coated with a blocking layer solution containing a mixture of 6.5 grams of gamma aminopropyltriethoxy silane, 39.4 grams of distilled water, 2.08 grams of acetic acid, 752.2 grams of 200 proof denatured alcohol and 200 grams of heptane. This wet coating layer was then allowed to dry for 5 minutes at 135° C. in a forced air oven to remove the solvents from the coating and form a crosslinked silane blocking layer. The resulting blocking layer had an average dry thickness of 0.04 micrometer as measured with an ellipsometer.

An adhesive interface layer was then applied to the blocking layer with a coating solution containing 49000 polyester adhesive. The applied adhesive interface wet coating was dried for 1 minute at 125° C. in a forced air oven. The resulting adhesive interface layer had a dry thickness of about 0.05 micrometer.

The adhesive interface layer was then coated with a charge generating layer. The charge generating layer was coated from a dispersion of 3 weight percent sodium doped trigonal selenium, having particle sizes ranging from about 0.05 to about 0.2 micrometer, about 6.8 weight percent polyvinyl carbazole, and 2.3 weight percent N,N'-diphenyl-N,N'-bis[3-methylphenyl]-[1,1'-biphenyl]4,4'-diamine in a 1:1 ratio by volume mixture of THF and toluene. This resulting slurry solution was thereafter coated onto the adhesive interface layer and dried for 2 minute at 135° C. in a forced air oven to give a dried charge generating layer of 2.5 micrometer in thickness. A strip of about 10 millimeters wide along one edge of the substrate web stock bearing the blocking layer and the adhesive layer was deliberately left uncoated to facilitate adequate electrical contact by a ground strip layer to be applied later.

This coated web stock was then cut and divided into six sample webs. Each of the sample web was simultaneously coated over with a charge transport layer (containing 5, 10, 20, 30, 40, or 50 weight percent of charge transport compound based the weight of the charge transport layer) and a ground strip layer by a co-coating method. Six charge transport layer solutions were each prepared by introducing into an amber glass bottle with MAKROLON 5705®, a Bisphenol A polycarbonate thermoplastic having a molecular weight of about 120,000 commercially available from Farbensabriken Bayer A.G. and N,N'-diphenyl-N,N'-bis[3-methylphenyl]-1,1'-biphenyl-4,4'-diamine (m-TBD). The contents in amber glass bottles were each dissolved to give a 15 percent by weight solid in methylene chloride. The prepared solutions, having the six different m-TBD concentration, were applied onto the charge generating layer of each respective sample web to form a coating which upon drying in a forced air oven gave a charge transport layer 24 micrometers thick.

The strip, about 10 millimeters wide, of the adhesive layer left uncoated by the charge generator layer, was coated with a ground strip layer during the co-extrusion process. The ground strip layer coating mixture was prepared by combining 23.81 grams of polycarbonate resin (MAKROLON® 5705, 7.87 percent by total weight solids, available from Bayer A.G.), and 332 grams of methylene chloride in a carboy container. The container was covered tightly and placed on a roll mill for about 24 hours until the polycarbonate was dissolved in the methylene chloride. The resulting solution was mixed for 15-30 minutes with about 93.89 grams of graphite dispersion (12.3 percent by weight solids) of 9.41 parts by weight of graphite, 2.87 parts by weight of ethyl cellulose and 87.7 parts by weight of solvent (Acheson Graphite dispersion RW22790, available from Acheson Colloids Company) with the aid of a high shear blade dispersed in a water cooled, jacketed container to prevent the dispersion from overheating and losing solvent. The resulting dispersion was then filtered and the viscosity was adjusted with the aid of methylene chloride. This ground strip layer coating mixture was then applied along with the charge transport layer to form an electrically conductive ground strip layer having a dried thickness of about 14 micrometers. Each of the six imaging member web stocks containing all of the above layers was then passed through 125° C. in a forced air oven for 3 minutes to simultaneously dry both the charge transport layer and the ground strip.

An anti-curl coating was prepared by combining 88.2 grams of polycarbonate resin (MAKROLON® 5705), 7.12 grams Vitel PE-200 copolyester (available from Goodyear Tire and Rubber Company) and 1,071 grams of methylene chloride in a carboy container to form a coating solution containing 8.9 percent solids. The container was covered tightly and placed on a roll mill for about 24 hours until the polycarbonate and polyester were dissolved in the methylene chloride to form the anti-curl back coating solution. The anti-curl back coating solution was then applied to the rear surface (side opposite the charge generating layer and charge transport layer) of each electrophotographic imaging member web and dried to a maximum temperature of 125° C. in a forced air oven for 3 minutes to produce a dried coating layer having a thickness of 14 micrometers and render imaging member flatness. The fabricated imaging members containing 5, 10, 20, 30, 40, or 50 weight percent of m-TBD in the charge transport layer served as reference imaging members.

## REFERENCE EXAMPLE II

Three electrophotographic imaging members were prepared as described in Reference Example I, except the charge transport layer was prepared from one of three different hole transporting polymers. The charge transport layer was still 24 microns thick.

The first hole transport polymer was a film forming polyvinyl carbazole commercially available from BASF Corporation. The molecular structure of the hole transport polymer polyvinyl carbazole is shown below:



The second hole transporting polymer was a polyester homopolymer having intrinsic hole transport capability. This polyester homopolymer comprised an ester linkage to the meta position of an aryl diamine hole transport compound as that described in Formula 1. The meta linkage polyester homopolymer had the following molecular structure:



The third hole transporting polymer was a polyester homopolymer having intrinsic hole transport capability, except that the ester linkage was to the para position of the hole transport compound. The para linkage polyester homopolymer had the following molecular structure:



#### Electrophotographic Measurement

The six imaging members of Reference Example I and the three imaging members of Reference Example II were each evaluated for key photo-electrical properties using a xerographic scanner. The scanner comprised a 3.25-inch cylindrical aluminum drum, a corotron device, an exposure/erase lamp, and probes mounted around the periphery of the drum. The imaging members were taped onto the drum and the drum was then set to rotate at a constant speed of 3.43 inches per second. In essence, the test was carried out by first resting the imaging members in the dark overnight prior to charging. Each member was negatively charged by the corona device in the dark to a development potential of -800 volts and then discharged by the exposure/erase lamp to about 250 erg/cm<sup>2</sup> of light energy. Thereafter, the imaging members were each subsequently subjected to the equivalent life test of 100 imaging cycles. The surface potential  $E_O$  and residual voltage  $E_R$  of each imaging member measured after 100 cycles and the values thus obtained were recorded for comparison.

The surface potential  $E_O$  and residual voltage  $E_R$  for the imaging members of Reference Example I were plotted and are shown in FIG. 4. The measurements were made with a probe, adjacent to the imaging member and the corotron, at 0.3 second after charging. The probe was connected to a

Keithly 610B Electrometer and the output of which was transmitted to a Model 7402A Hewlett Packard Recorder. As shown in FIG. 4, the imaging members having 50 and 40 weight percent m-TBD gave equivalent surface potential  $E_O$  and residual voltage  $E_R$ . However, reducing m-TBD below 30 weight percent showed a significant deterioration in field

strength. In other words, the imaging members containing 20, 10, and 5 weight percent m-TBD were not satisfactory for xerographic use.

The three imaging members of Reference Example II showed marginally acceptable photo-electrical function. The

polyvinyl carbazole charge transport layer functioned, at best, like an imaging member containing 27 weight percent m-TBD. The charge transport layer using either polyester homopolymers functioned like an imaging member containing about 38 weight percent m-TBD.

#### CONTROL EXAMPLE

An electrophotographic imaging member was prepared by providing a 0.02 micrometer thick titanium layer coated on a biaxially oriented polyethylene naphthalate substrate (Kaledex™ 2000) having a thickness of 3.5 mils (0.09 millimeters).

Applied thereon with a gravure applicator, was a solution containing 50 grams 3-amino-propyltriethoxysilane, 41.2 grams water, 15 grams acetic acid, 684.3 grams of 200 proof denatured alcohol and 200 grams heptane. This layer was then dried for about 2 minutes at 120° C. in the forced air drier of the coater. The resulting blocking layer had a dry thickness of 500 Angstroms.

An adhesive layer was then prepared by applying a wet coating over the blocking layer, using a gravure applicator, containing 0.2 weight percent of polyarylate adhesive (Ardel™ D100 available from Toyota Hsutsu Inc.) in a 60:30:10 volume ratio mixture of tetrahydrofuran/monochlorobenzene/methylene chloride. The adhesive layer was then dried

29

for about 2 minutes at 120° C. in the forced air dryer of the coater. The resulting adhesive layer had a dry thickness of 200 Angstroms.

A photogenerating layer dispersion was prepared by introducing 0.45 grams of Lupilon200™ (PC-Z 200) available from Mitsubishi Gas Chemical Corp and 50 ml of tetrahydrofuran into a 100 gm glass bottle. To this solution was added 2.4 grams of hydroxygallium phthalocyanine and 300 grams of  $\frac{1}{8}$  inch (3.2 millimeter) diameter stainless steel shot. This mixture was then placed on a ball mill for 8 hours. Subsequently, 2.25 grams of PC-Z 200 was dissolved in 46.1 gm of tetrahydrofuran, and added to this OHGaPc slurry. This slurry was then placed on a shaker for 10 minutes. The resulting slurry was, thereafter, applied to the adhesive interface with a Bird applicator to form a charge generation layer having a wet thickness of 0.25 mil (about 6 microns). A strip about 10 mm wide along one edge of the substrate web bearing the blocking layer and the adhesive layer, was deliberately left uncoated to facilitate adequate electrical contact by the ground strip layer that was to be applied later. The charge generation layer was dried at 120° C. for 1 minute in a forced air oven to form a dry charge generation layer having a thickness of 0.4 micrometers.

This charge generation layer was coated over with a first (bottom) charge transport layer. The charge transport layer was prepared by introducing into an amber glass bottle N,N'-diphenyl-N,N'-bis(3-methylphenyl)-[1,1'-biphenyl]-4,4'-diamine and a polymer binder of MAKROLON® 5705, a bisphenol A polycarbonate, poly(4,4'-isopropylidene diphenyl)carbonate, or poly(4,4'-diphenyl)-1,1'-cyclohexane carbonate in a weight ratio of 50:50. The resulting mixture was dissolved to produce a solution of 15 weight percent solids, in 85 weight percent methylene chloride. This solution was applied onto the photogenerator layer to form a coating which upon drying gave a dried first charge transport layer thickness of 14.5 micrometers.

A second (top) charge transport layer having a dry thickness of 14.5 microns was then coated onto the first charge transport layer in the same manner. This formed a dual charge transport layer having a total dried thickness of 29 micrometers. Each layer comprised 50 weight percent hole transport compound and 50 weight percent of polymer binder.

The approximately 10 millimeter wide strip of the adhesive layer left uncoated by the photogenerator layer was coated over with a ground strip layer during the application of the second charge transport by co-coating process. This ground strip layer, after drying along with the co-coated charge transport layer at 135 degrees Celsius in a forced air oven for 5 minutes, had a dried thickness of about 19 micrometers. This ground strip was electrically grounded, by conventional means such as a carbon brush contact means during conventional xerographic imaging process.

An anticurl layer coating was prepared by combining 8.82 grams of polycarbonate resin (MAKROLON® 5705, available from Bayer AG), 0.72 grams of polyester resin (VITEL PE-200, available from Goodyear Tire and Rubber Company) and 90.1 grams of methylene chloride in a glass container to form a coating solution containing 8.9 weight percent solids. The container was covered tightly and placed on a roll mill for about 24 hours until the polycarbonate and polyester were dissolved in the methylene chloride to form the anticurl coating solution. The anticurl coating solution was then applied to

30

the rear surface (side opposite the photogenerator layer and charge transport layer) of the imaging member web stock, again by extrusion coating process, and dried at 135 degrees Celsius for about 5 minutes in the forced air oven to produce a dried film thickness of about 17 micrometers. The prepared imaging member had a material configuration as shown in FIG. 1, but without an overcoat, and served as a control.

## COMPARATIVE EXAMPLE

10

A comparative electrophotographic imaging member web was prepared as described in the Control Example, except that the 14.5-micrometer thick first charge transport layer of the dual charge transport layer was replaced by a layer consisting of 30 weight percent N,N'-diphenyl-N,N'-bis(3-methylphenyl)-1,1'-biphenyl-4,4'-diamine and 70 weight percent MAKROLON 5705™. The ratio of charge transport molecules in the first layer to that in the second layer was 30:50, or 60 percent.

## Photo-Electrical Property and CDS Assessment

The imaging members of the Control Example and the Comparative Example were tested for their xerographic sensitivity and cyclic stability in a scanner. In the scanner, each imaging member cut sheet to be evaluated was mounted on a cylindrical aluminum drum substrate, which was rotated on a shaft. The devices were charged by a corotron mounted along the periphery of the drum. The surface potential was measured as a function of time by capacitatively coupled voltage probes placed at different locations around the shaft. The probes were calibrated by applying known potentials to the drum substrate. Each imaging member cut sheet on the drum was exposed to a light source located at a position near the drum downstream from the corotron. As the drum was rotated, the initial (pre-exposure) charging potential (V<sub>ddp</sub>) was measured by a first voltage probe. Further rotation led to an exposure station, where the photoreceptor device was exposed to monochromatic radiation of a known intensity of 3.5 ergs/cm<sup>2</sup> to obtain V<sub>bg</sub>. The devices were erased by a light source located at a position upstream of charging to obtain V<sub>r</sub>. The results obtained from the measurements listed in Table 1 below include the charging of each imaging member sheet in a constant current mode. The devices were charged to a negative polarity corona. The surface potential after exposure (V<sub>bg</sub>) was measured by a second voltage probe. In the design, the exposure could be turned off in certain cycles. The voltage measured at the second probe is then V<sub>ddp</sub>. The voltage generally is higher at the charging station. The difference between the charged voltage at the charging station and the V<sub>ddp</sub> is dark decay. The devices were finally exposed to an erase lamp of appropriate intensity and any residual potential (V<sub>r</sub>) was measured by a third voltage probe. After 10,000 charge-erase cycles, the V<sub>bg</sub> was remeasured and the difference between V<sub>bg</sub> for the first cycle and V<sub>bg</sub> for cycle 10,000 (ΔV<sub>bg</sub> 10K) was computed.

TABLE 1

| Example     | V <sub>bg</sub> (initial)<br>3.5 erg/cm <sup>2</sup> ;<br>V <sub>ddp</sub> = 500 | V <sub>bg</sub> (10k)<br>3.5 erg/cm <sup>2</sup> ;<br>V <sub>ddp</sub> = 500 | V <sub>r</sub><br>(300 erg/cm <sup>2</sup> ) | Dark<br>Decay |
|-------------|----------------------------------------------------------------------------------|------------------------------------------------------------------------------|----------------------------------------------|---------------|
|             |                                                                                  |                                                                              |                                              |               |
| CONTROL     | 57                                                                               | 92                                                                           | 20                                           | -193          |
| COMPARATIVE | 70                                                                               | 115                                                                          | 35                                           | -152          |

31

The imaging member cut sheets were then further tested with a floating probe scanner (FPS scanner) for Charge Deficient Spots (CDS) defects in a manner similar to that described in U.S. Pat. Nos. 6,008,653 and 6,119,536, incorporated herein by reference. All the imaging member cut sheets were mounted on a drum of the FPS scanner one at a time. The drum was rotated continuously and underwent a sequence of charging under a scorotron to about 700 volts. Then measurements of micro defects were made. These consisted of high resolution voltage measurements of from about 50 to about 100 micron resolution by an aerodynamically floating probe which was capacitively coupled to the imaging member charged surface. The probe was maintained at a constant distance of 50 microns during the entire scan of the sample surface. After this, the imaging member was discharged by an erase lamp before the next cycle started. In each cycle the drum was moved translationally in small steps of from about 25 to about 50 micrometers. The floating probe scanner then counted the CDS's over an area of about 100 to about 150 cm<sup>2</sup> and provided an average value/cm<sup>2</sup> to give results shown in Table 2 below.

TABLE 2

| EXAMPLE     | CDS count/cm <sup>2</sup> |
|-------------|---------------------------|
| CONTROL     | 13                        |
| COMPARATIVE | 3.2                       |

The data in Tables 1 and 2 indicate that an imaging member prepared with 30 weight percent m-TBD in the first layer and 50 weight percent m-TBD in the second layer did not suffer significant degradation in the resulting imaging member, but effectively suppressed CDS defects print out defects compared to the control imaging member.

## DISCLOSURE EXAMPLE

Three imaging members of the present disclosure may be prepared as described in the Control Example. However, the

32

first charge transport layers of these three members are prepared with the three hole transport polymers as shown in Reference Example II, one polymer per member. The resulting first charge transport layers are all 14.5 microns thick.

While particular embodiments have been described, alternatives, modifications, variations, improvements, and substantial equivalents that are or may be presently unforeseen may arise to applicants or others skilled in the art. Accordingly, the appended claims as filed and as they may be amended are intended to embrace all such alternatives, modifications variations, improvements, and substantial equivalents.

The invention claimed is:

1. An imaging member comprising:  
a substrate;  
a charge generating layer;  
a charge transport layer disposed about the charge generating layer; and  
a barrier layer disposed between the charge generating layer and the charge transport layer, wherein the barrier layer comprises a non-conducting or conducting film forming polymeric binder material.

2. The imaging member of claim 1, wherein the barrier layer comprises a non-conducting film forming polymeric binder material and contains no charge transport molecules.

3. The imaging member of claim 1, wherein the barrier layer contains from about 0 to about 20 weight percent of a charge transport molecule.

4. The imaging member of claim 1, wherein the barrier layer contains from about 3 to about 10 weight percent of a charge transport molecule.

5. The imaging member of claim 1, wherein the barrier layer has a thickness of from about 1 to about 2 microns.

6. The imaging member of claim 1, wherein the conducting film forming polymeric binder material of the barrier layer is selected from the group consisting of:

a polyester homopolymer having the structure of:



33

wherein x is from 2 to 20 and m is the degree of polymerization;

an organopolyphosphazene selected from the following four structures:



wherein R is selected from a pendant group having intrinsic 20 hole transport capability and y is the degree of polymerization;

34 a carbazole polymer having the structure of:



wherein R<sub>1</sub> is selected from



wherein n is the degree of polymerization; and R<sub>2-5</sub> are independently selected from H, alkyl, substituted alkyl, alkoxy, and the like and combinations thereof;

a polyester homopolymer having the structure of:



a hole transport compound-urethane copolymer, a fluorine-based pendant active moiety of a polyester, a fluorine-based active moiety polycarbonate, and a fluorine based active moiety polyurethane.

50 wherein x is from 2 to 20 and m is the degree of polymerization;

an organopolyphosphazene selected from the following four structures:

7. An imaging member comprising:

a substrate;

a charge generating layer;

a first charge transport layer adjacent to the charge generating layer and comprising a film forming polymer having inherent hole transporting capability; and

a second charge transport layer disposed upon the first charge transport layer, the second layer comprising a polymer binder and a charge transport material;

60 wherein the film forming polymer of the first charge transport layer is selected from the group consisting of:



35

wherein R is selected from a pendant group having intrinsic hole transport capability and y is the degree of polymerization;

a hole transport compound-urethane copolymer, a fluorine-based pendant active moiety of a polyester, a fluorine-based active moiety polycarbonate, and a fluorine based active moiety polyurethane.

8. The imaging member of claim 7, wherein the first charge transport layer has a thickness of from about 120 percent to about 40 percent of the thickness of the second charge transport layer.

9. The imaging member of claim 7, wherein the first charge transport layer contains no charge transport molecules.

10. The imaging member of claim 7, wherein the first charge transport layer further comprises a second film forming polymer having inherent hole transporting capability.

11. The imaging member of claim 7, further comprising a third charge transport layer disposed upon the second charge transport layer, the third layer comprising a polymer binder and a charge transport component, wherein the concentration of charge transport component in the third layer is from about 1 to about 95 percent of the concentration of charge transport material in the second layer.

12. The imaging member of claim 11, wherein the polymer binder in both second and third charge transport layers is poly(4-4'-isopropylidene diphenyl carbonate) or poly(4,4'-diphenyl-1-1'-cyclohexene carbonate).

13. The imaging member of claim 11, wherein the third charge transport layer comprises a charge transport molecule in a concentration lower than the concentration of charge transport material in the second layer.

36

14. The imaging member of claim 13, wherein the total amount of charge transport compound in both the second and third charge transport layers is from about 45 to about 75 weight percent, based on the total weight of all charge transport layers.

15. The imaging member of claim 13, wherein the first charge transport layer is between about 120 percent and about 40 percent the total thickness of both second and third charge transport layers.

16. The imaging member of claim 7, wherein the second charge transport layer contains an additive selected from the group consisting of antioxidant, nanoparticle dispersion, surfactant, and light shock resisting agent.

17. An imaging member comprising:  
a substrate;  
a charge generating layer;  
a first charge transport layer, the first layer comprising a first polymer binder and a charge transport material;  
a second charge transport layer disposed upon the first charge transport layer, the second layer comprising a second polymer binder and a charge transport material;  
and

a barrier layer located between the charge generating layer and the first charge transport layer;  
wherein the barrier layer comprises a hole transporting film forming polymeric binder material; and  
wherein the film polymer binder is selected from the group consisting of:  
a carbazole polymer;  
a polyester homopolymer having the structure of:



or



37

wherein x is from 2 to 20 and m is the degree of polymerization;  
an organopolyphosphazene selected from the following four structures:



wherein R is selected from a pendant group having intrinsic hole transport capability and y is the degree of polymerization;

a hole transport compound-urethane copolymer, a fluorine-based pendant active moiety of a polyester, a fluorine-based active moiety polycarbonate, and a fluorine-based active moiety polyurethane.

**18.** The imaging member of claim 17, wherein the barrier layer contains no charge transport molecules.

38

**19.** The imaging member of claim 17, wherein the first charge transport layer further comprises a first charge transport component in the amount of from about 10 to about 35 weight percent, by weight of the first charge transport layer.

**20.** The imaging member of claim 17, wherein the first charge transport layer has a thickness of from about 120 percent to about 40 percent of the thickness of the second charge transport layer.

**21.** The imaging member of claim 17, wherein the first charge transport layer and the second charge transport layer have the same polymer binder.

**22.** The imaging member of claim 21, wherein the polymer binder is a polycarbonate.

**23.** The imaging member of claim 22, wherein the polycarbonate binder in both the first charge transport layer and the second charge transport layer is poly(4-4'-isopropylidene diphenyl carbonate) or poly(4,4'-diphenyl-1,1'-cyclohexene carbonate).

**24.** The imaging member of claim 17, wherein the second charge transport layer contains an additive selected from the group consisting of antioxidant, nanoparticle dispersion, surfactant, and light shock resisting agent.

\* \* \* \* \*